

Jan. 3, 1933.

W. H. WOODFORD

1,892,759

AMMUNITION

Filed March 19, 1930



*Fig. 1*



*Fig. 2*



*Fig. 3*

INVENTOR.

*Watson H. Woodford*  
BY *A. G. Kline*  
*A. D. White*  
ATTORNEYS.

## UNITED STATES PATENT OFFICE

WATSON H. WOODFORD, OF BRIDGEPORT, CONNECTICUT, ASSIGNOR TO REMINGTON ARMS COMPANY, INC., A CORPORATION OF DELAWARE

AMMUNITION

Application filed March 19, 1930. Serial No. 436,988.

The present invention relates to projectiles and has for its principal object the provision of a projectile which, during its passage through the bore of the gun, will leave on the 5 wall of the gun bore a coating or film which will effectively protect the bore against corrosion even under the most adverse conditions of humidity and temperature.

It is a further object of the present invention to provide a projectile coated with a material which presents a dry surface and is at the same time highly effective as a lubricant for the projectile during its passage 10 through the bore of the gun. The necessity for using such a lubricant as grease, which 15 possesses many disadvantages, is thereby dispensed with.

It is a further object of the present invention to provide a projectile coated with a 20 material presenting a highly lustrous and attractive finish, and which, in addition, is not susceptible to rapid oxidation or corrosion, and which therefore gives good protection 25 against deterioration of the projectile itself.

The evil known as "after-corrosion" in 30 gun barrels has for a long time been a troublesome problem. As is well known, any steel surface on exposure to the atmosphere will 35 rust, and this is likewise true in connection with the steel surface exposed in the bores of guns. By "after-corrosion" is meant the 40 corrosion which occurs in the bores of guns after shooting, the activity of which corrosion has been greatly augmented heretofore 45 by the deposit, in the bores of the guns, of 50 residues from some types of ammunition when fired in the guns. This has been especially true in the past where ammunition priming mixtures were used containing such 55 an ingredient as potassium chlorate, which 60 leaves hygroscopic residues in the gun bore, which residues become lodged in the fissures and tool wounds of the bore surface, and which attract moisture from the atmosphere, 65 in the presence of which a ravaging corrosion 70 of the steel of the bore takes place.

Efforts to overcome after-corrosion have 75 for the most part been directed toward the discovery of ingredients for the explosive 80 constituents of ammunition which would not

only satisfy the rigid ballistic and stability requirements, but would, in addition, leave no residues of a hygroscopic nature, and which would therefore assist in preventing 55 after-corrosion in gun bores. Such ammunition has been successfully produced and used, but it is to be noted that this ammunition does not in a positive manner "prevent" 60 corrosion in the gun bore, inasmuch as it does not leave a protective coating in the bore of 65 the gun, but merely is not capable of leaving objectionable residues of a nature which might promote corrosion.

Further methods of combating the evil of 70 after-corrosion have involved the provision 75 of certain ingredients in the explosive constituents of ammunition which appear to react with the material forming the bullet surface to actually form a corrosion preventive 80 film in the bore of the gun in which the ammunition is fired. Such ammunition has been produced and used with success, but in this ammunition the available range in the choice of explosive ingredients, which will 85 successfully attain these results is quite limited. It is obviously highly desirable that ammunition be produced which is capable of preventing corrosion in the gun bore without the necessity thereby of limiting the range 90 in the choice and selection of successfully operative ingredients for the explosive constituents of this ammunition. Furthermore, in this ammunition the bore coating characteristics appear to be dependent upon the joint use of particular explosive ingredients, together 95 with a bullet having a surface of a particular material. In connection with this ammunition tests have indicated that success in forming a protective coating in the gun bore is apparently due to some form of reaction 100 between the explosive ingredients and bullet material. It is desirable that corrosion preventive ammunition be produced in which any of the common types of projectiles, already in use, may be utilized, and in which the successful formation of a bore protective coating may be effected without dependence upon any form of reaction between the ingredients of the ammunition and the material of the projectile. The present invention aims

as an additional object to obtain these results.

Besides offering a solution for the problem of corrosion in gun bores the present invention aims also to lessen in a large degree the pernicious effects known as "metal fouling". In metal fouling, fragments of metal are torn from the bullet and deposited as isolated patches in the gun bore, and as repeated firings take place this fouling accumulates, resulting in impaired accuracy, reduction of bore diameter, as well as rendering the gun unsafe. Grease has been much used as a lubricant on bullets to prevent metal fouling, but the use of grease is attended by many serious disadvantages, such as the difficulty of retaining the grease on the projectile and the undesirable accumulation of foreign matter by the grease. Various so-called dry lubricants have been proposed, most of which constitute a soft metal applied as a jacket or deposit on the projectile. The present invention contemplates the provision of a projectile coated with a metal which not only functions to prevent bore corrosion but also constitutes a dry lubricant of superior bullet lubricating qualities and which very effectively acts to prevent metal fouling.

According to the present invention the hereinbefore mentioned and still further objects are fulfilled, as will be apparent from the following specification, by the application of the metal cadmium to projectiles, preferably in the form of coatings applied to the surfaces of the projectiles.

The natural corrosion preventive properties of cadmium are well known. A cadmium coating on a steel surface is known to be highly efficient in protecting the steel against rust, this coating being superior in many respects to coatings of other metals which have been long used for rust prevention, such for example as zinc and tin. The element cadmium stands near the element iron in the electromotive series and will not deteriorate as rapidly from anodic attack as other metals more remote from iron in the series. At the same time, cadmium is electro-positive with respect to iron and will protect iron in accordance with well established electro-chemical principles. The utilization of these and other well known desirable properties of cadmium is contemplated in connection with the present invention. In addition, the discovery of heretofore unknown properties of cadmium is involved as an important phase of the invention.

It has been discovered in connection with experiments leading to the present invention that new and highly advantageous results are obtained when projectiles coated with cadmium are fired in guns. A gun barrel having such projectiles fired therein is found to be left with a highly lustrous coating on the walls of the bore. The coating or film

thus formed is very thin and is uniformly distributed throughout the bore. This film fills the microscopic fissures and tool wounds in the steel of the bore and prevents accumulation of hygroscopic residues which would attract and hold moisture and thereby promote corrosion. At the same time the film serves to act as a bar against contact of the steel with the atmosphere and thus, in a positive manner, actually prevents corrosion of the bore surface. In addition, considering the electrochemical properties heretofore mentioned, the higher electrode potential of cadmium in the electromotive series causes the cadmium to guard the bore steel against galvanic attack, and at the same time the proximity of cadmium in the series assures the cadmium against rapid deterioration by anodic attack. Tests have demonstrated that gun barrels, after having a few cadmium plated bullets shot therein, are capable of withstanding exposure to severe atmospheric conditions without a sign of corrosion in the bore. In one instance, several cartridges having cadmium plated bullets were fired in a barrel, and this barrel was then placed in a chamber of heated and highly humidified air. After confinement of this barrel to this chamber for a period of over two weeks, examination showed the bore to be bright and entirely free from rust, while parts of the barrel, other than the bore, were found to be heavily rusted. This test was carried on in its entirety without in any way cleaning or treating the bore of the barrel, other than applying cadmium as above described. Repeated firing of cadmium plated bullets in a gun has shown that the protective coating or film in the bore remains thin and uniformly distributed, and that the diameter of the bore is not materially altered even after a large number of bullets have passed through the bore.

The projectile may be provided at its surface with cadmium by any suitable means. The projectile may be dipped into a molten bath of cadmium, if desired. Or, the molten cadmium may be applied to the projectile as by spraying; or the coating may be formed by electrical deposition, or by any other suitable depositing method. Further, the coating may be applied as a previously formed jacket, plate or band, etc., if desired. Inasmuch as electrical deposition affords a means whereby the thickness of the coating may be easily controlled, and as only a very thin coating of cadmium is required to perform the desired results successfully, I prefer to coat the projectiles by this method. The well-known electrical "barrel plating" process, utilizing a cadmium cyanide solution, constitutes a very suitable plating method for accomplishing the purposes of the present invention.

The entire surface of the projectile may

be cadmium plated, thereby causing the projectile to present an attractive surface over its entire area. After plating with cadmium, the surface may be polished or finished in any suitable manner, thus providing a bright surface which is found to be capable of holding its lustre over a long period of time. It will be understood, however, that it is not essential to coat the entire surface of the projectile with cadmium, but that the above described bore coating effects may be obtained by providing cadmium on only such portions of the projectile which engage the rifling of the gun or which contact the bore surface. In projectiles of the type having rifling bands formed thereon the cadmium may be confined to the rifling band only, if desired. I prefer, however, to coat the entire projectile in order to obtain the attractive finish as well as the protection to the projectile itself, which cadmium affords.

It will be understood also, as mentioned above, that the cadmium may be applied to the projectile as a previously formed jacket, if desired, after methods known in the art in connection with jackets of other materials. However, due to the fact that but a very thin coating of cadmium is required, and for the sake of economy, it is preferred to apply the cadmium to the projectile by some form of depositing process.

In the drawing, which forms a part of this specification, there are illustrated on an enlarged scale several representative types of projectiles embodying the present invention.

In Fig. 1 is shown in elevation, partly in section, one type of projectile embodying the invention.

In Fig. 2 is shown a similar view of another type of projectile embodying the present invention.

In Fig. 3 is shown a similar view of still another type of projectile embodying the present invention.

The projectile of Fig. 1 is a standard lead bullet of the type popularly used with small calibre ammunition, such as for the .22 calibre rifle. The bullet proper, indicated at 10, is formed of lead, and a rifle band 11, is formed on its outer surface integral with the body of the bullet. The entire surface of the bullet is provided with a thin coating or plating 12 of cadmium, which besides serving in the capacity of forming a protective coating in the gun bore, serves also as a protective coating of attractive appearance for the bullet itself.

The projectile illustrated in Fig. 2 is a rifle bullet of the mushrooming type. A jacket 13, of copper, gilding metal, or other metal or alloy, is filled with a core 14 of lead or material having high percentage of lead. The nose of this projectile is provided with an aperture 15, and the jacket to the rear of this aperture is weakened as at 16 to facili-

tate mushrooming of the projectile on striking an object. The whole projectile including the interior of the aperture is plated with a thin coating 17 of cadmium. The coating being very thin and the metal cadmium being sufficiently soft, the mushrooming qualities of this bullet are not materially affected, while at the same time the many advantageous results to be obtained from a cadmium coating, as hereinbefore pointed out, are at the same time obtained.

In Fig. 3, there is shown a rifle bullet of the ordinary jacketed type. A jacket 18, of copper, gilding metal, cupro-nickel or other metal or alloy, surrounds a core 19 of lead or metal having a high percentage of lead. The whole outer surface is provided with a thin coating 20 of cadmium.

It will be obvious that a similar coating of cadmium may be provided on many types of projectiles other than the three types illustrated, and that like benefits may be obtained from such provision. The term "projectile" as used in the specification and following claim is used generically and is to be understood as referring to projectiles generally, including projectiles for ordnance, bullets for small arm rifles and smooth bore guns, as well as ball-shot. The bore coating properties of cadmium are apparently entirely independent of any reaction of this metal with any of the explosive constituents of ammunition, and therefore cadmium coated projectiles may be successfully used in conjunction with ammunition generally regardless of the accompanying explosive constituents of the ammunition.

Although the invention has been described with reference to cadmium alone as a coating in the form of a plating, it is to be understood that various forms of cadmium amalgams and cadmium alloys may be used as alternatives if desired. It has been found that excellent results are to be obtained from cadmium alone, and that it is unnecessary to complicate the process of coating by introducing other materials.

In the specification and following claim the terms "coated" with cadmium and "coating" of cadmium are used as referring to a material containing cadmium, either alone or alloyed with other materials, constituting a portion only, or the entire surface of a projectile; and these terms refer to the application of such coating by any known means, including application by previously formed jackets, bands, etc., or by any suitable manner of depositing the coating on the projectile, or by alloying the coating with the material of the projectile.

It is to be understood that the embodiments of the present invention as shown and described are purely illustrative, and that the scope of the invention is not to be limited

thereby except insofar as is defined in the following claim.

I claim:

5 A projectile having applied thereto a coating of cadmium capable of forming a corrosion preventive film on the walls of a gun bore when the projectile is fired therein.

WATSON H. WOODFORD.

10

15

20

25

30

35

40

45

50

55

60

65